

March 10, 1925.

1,529,249

H. D. GUE

METHOD OF AND APPARATUS FOR ELECTRODEPOSITION AND THE PRODUCT THEREOF

Filed May 19, 1923



INVENTOR:

Harry D. Gue

BY

James L. Stewart

his ATTORNEY.

## UNITED STATES PATENT OFFICE.

HARRY D. GUE, OF BROOKLYN, NEW YORK.

## METHOD OF AND APPARATUS FOR ELECTRODEPOSITION AND THE PRODUCT THEREOF.

Application filed May 19, 1923. Serial No. 640,036.

*To all whom it may concern:*

Be it known that I, HARRY D. GUE, a citizen of the United States, and a resident of the borough of Brooklyn, county of Kings, and State of New York, have invented certain new and useful Improvements in Methods of and Apparatus for Electrodeposition and the Product Thereof, of which the following is a specification.

10 This invention has reference to the art of electro-metallurgy and particularly relates to an improved process of electro-deposition, which has many advantages in technical results, to an improved product, resulting from said method, which has several important and novel characteristics and to an apparatus for carrying out said method and by which the said product is effected, economically, efficiently, and with unusual facility.

15 This invention may be aptly illustrated by reference to a conventional form of electro-deposition, wherein a container or vat is provided to contain a suitable electrolyte, in which are immersed an anode and a cathode; these are usually included in a circuit carrying a direct current and the electro-deposition is accomplished by reason of the liberation of particles from one of said electrodes, and the deposit of the same on the other electrode, or the releasing of said particles to enrich the electrolyte, all according to well-known principles of electrodeposition. Reference in the claims to "an electrolytic apparatus" is intended to include and identify an apparatus substantially the same as that above described.

20 In accordance with the several branches of my invention, an apparatus is employed in which, in addition to the usual electrolytic pair, one or more extra electrodes are used which are capable of transmitting an electric current; but, preferably, the extra electrode is of non-resolvable character or quality.

25 The drawings accompanying this specification show diagrammatically various ways in which I contemplate applying my invention and carrying out my method, details of which will now be set forth.

30 In the several figures, the container or vat is indicated by the numeral 1, which contains any suitable electrolyte indicated at 2. In all the figures the anode is indicated

35 by A, the cathode by C, and the extra electrodes by A' and A'', and it will be understood that one, or a plurality of, extra electrodes may be employed, which may be of carbon, or other insoluble material. Two or more extra electrodes may be employed 40 without departing from the spirit of my invention. The extra electrodes are so-called "idle electrodes" and are not primarily intended to be dissolved in the electrolyte to enrich the same, or to be deposited upon the 45 object to be coated. Where resolvable electrodes are employed, the fact of such resolvable quality does not appear to seriously affect the result; for, apparently, a negative result is obtained and it is assumed that 50 where particles are released under one phase of the current, they are restored under the opposite phase thereof.

55 In the several figures, the alternating current generator or source of alternating current is indicated at 3, and the direct current generator or source of direct current is indicated at 4. I have also indicated the same as D. C. and A. C.

60 In Figure 1, the anode and cathode are connected to the opposite poles of a source of direct current, in usual manner, by the leads 5 and 6; while the source of alternating current has one of its leads 7 connected to the cathode and its other lead 8 connected 65 to the independent electrode, which may be formed of non-resolvable material, is a conductor of current, and may be made of carbon or other suitable material.

70 In Figure 2, the anode is connected by lead 9 to one pole of the D. C. generator, the opposite pole of which is connected by lead 10 to the cathode; while one pole of the A. C. generator is connected by lead 11 to the anode and the opposite pole is connected by 75 lead 12 to the independent electrode.

75 In Figure 3, the anode is connected by lead 13 to one pole of an A. C. generator, the opposite pole of which is connected by lead 14 to the independent electrode. In 80 this form of my invention, the anode is also connected by lead 15 to one pole of a D. C. generator, the opposite pole of which is connected by a lead 16 to the cathode. Also, the cathode is connected by lead 17 to one 85 pole of a second A. C. generator, the opposite pole of which is connected by lead 18 to the independent electrode.

In Figure 4, the anode is connected by lead 19 to one pole of an A. C. generator, the opposite pole of which is connected by lead 20 to the independent electrode. In 5 this form the cathode is connected by lead 21 to one pole of a second A. C. generator, the opposite pole of which is connected by lead 22 with the independent electrode. Additionally, the cathode is connected by lead 10 23 to one pole of a D. C. generator, the opposite pole of which is connected by lead 24 to the anode.

In the form of my invention shown in Figure 5, the anode is connected by lead 15 25 to one pole of an A. C. generator, the opposite pole of which is connected by lead 26 to the cathode. The anode is also connected by lead 27 to one pole of a D. C. generator, the opposite pole of which is connected by lead 20 28 to the cathode. Additionally, the anode is connected by lead 29 to one pole of a second A. C. generator, the opposite pole of which is connected by lead 30 to the independent electrode.

25 In the Figure 6 form of my invention, the anode is connected by lead 31 to one pole of a D. C. generator, the opposite pole of which is connected by lead 32 to the cathode, the cathode in turn being connected by lead 33 30 to one pole of an A. C. generator, the opposite pole of which is connected by lead 34 to an independent electrode A'. The anode is also connected by lead 35 to one pole of a second A. C. generator, the opposite pole of 35 which is connected by lead 36 to a second independent electrode A''.

When two sources of alternating current are used in combination, as in Figures 3 to 40 6, inclusive, they may be of the same voltage and frequency or of different voltage and/or frequency; or they may be subdivisions of a multi-phase source of alternating current.

From the foregoing it will be seen that my method of electrolytic deposition involves the use of one or more independent electrodes having the characteristics described, the independent electrode or electrodes being immersed in the electrolyte, and acting only as a conductor for the alternating currents generated. And, as stated, the extra electrode may be, and preferably is, composed of non-resolvable material; but, I do not wish to be limited to electrodes of such characteristics, since I have obtained 55 good results from electrodes which are resolvable electro-chemically. Therefore, in certain of my claims limitation will not be made to the preferred characteristics of the extra electrode.

60 I have determined experimentally that the presence of the independent electrode or electrodes in the electrolyte, and connected to the generators in the manner indicated, results in increasing the speed of deposition and plating, increases the bond, or adher-

ence, between the deposited metal and the substances coated, secures a more dense and homogeneous deposit or coating, and thus greatly improves the product. Inasmuch as the explanation of the phenomena involved in the method and also in the operation of my apparatus is complex, and at best would be merely tentative, I do not deem it necessary herein to enter into a detailed statement of what I believe to be the probable explanation. Experimentation, however, has demonstrated the foregoing favorable conditions and results emanating from the method described and the arrangements and combinations of generators and electrodes. 70 75

Having thus described my invention, what I claim and desire to secure by Letters Patent is:

1. The herein described method of electro-deposition consisting of employing an electrolytic apparatus substantially as described and also employing in addition thereto an electrode immersed in the electrolyte and bringing said additional electrode and one of the usual pair of electrodes 80 85 into a common electric circuit of predetermined characteristic.

2. The herein described method of electro-deposition consisting of employing an electrolytic apparatus substantially as described and also employing in addition thereto an electrode immersed in the electrolyte and bringing said additional electrode and one of the usual pair of electrodes into a common electric circuit of alternating current. 90 95

3. The herein described method of electro-deposition consisting of employing an electrolytic apparatus substantially as described, and also employing a plurality of additional electrodes immersed in the electrolyte, and bringing said additional electrodes and the electrodes of said electrolytic apparatus into common electric circuits of predetermined characteristics. 100 105

4. In combination with an apparatus for electro-deposition including an electrolyte, an electrolytic pair in said electrolyte, an additional electrode immersed in said electrolyte, an electric circuit of predetermined characteristic in which the electrolytic pair is inserted and an independent electric circuit in which the additional electrode and one of the electrolytic pair are inserted. 110 115

5. In combination with an electrolytic tank containing the usual electrolyte and anode and cathode, a direct current circuit in which the anode and cathode are included, an independent electrode and an alternating current circuit in which the independent electrode and one of the electrolytic pair are inserted. 120

6. An article of manufacture having a coating of metal thereon produced by an electrolytic deposition process involving the use of the usual electrolytic pair, an inde- 125 130

pendent electrode inserted in an electric circuit of different characteristics conveyed to the electrodes through the electrolyte.

7. The herein described method of electro-deposition consisting in employing an electrolytic apparatus, substantially as described, and also employing an electrode of non-resolvable character immersed in the electrolyte, and bringing said non-resolvable electrode and one of the usual pair of electrodes into a common electric circuit of predetermined characteristics.

8. The herein described method of electro-deposition consisting in employing an electrolytic apparatus, substantially as described, and also employing an electrode of non-resolvable character immersed in the electrolyte, and bringing said non-resolvable electrode and one of the usual pair of electrodes into a common electric circuit of alternating current.

9. The herein described method of electro-deposition consisting in employing an electrolytic apparatus, substantially as described, and also employing a plurality of electrodes of non-resolvable character immersed in the electrolyte, and bringing said non-resolvable electrodes and the electrodes of the apparatus into common electric circuits of predetermined character.

10. In combination with an apparatus for electrodeposition including an electrolyte, an electrolytic pair in said electrolyte, and a non-resolvable electrode immersed in said electrolyte, an electric circuit of predetermined character in which the electrolytic

pair is inserted, and an independent electric circuit in which the non-resolvable electrode and one of the electrolytic pair are inserted.

11. In combination with an electrolytic cell, containing the usual electrolyte and anode and cathode, a direct current circuit in which the anode and cathode are inserted, an independent electrode of non-resolvable character, and an alternating current circuit in which the independent electrode and one of the electrolytic pair are inserted.

12. An article of manufacture having a coating of metal thereon produced by an electrolytic deposition process involving the use of the usual electrolytic pair, and an independent electrode inserted in an electric circuit of different characteristics conveyed to the electrodes through the electrolyte.

13. An article of manufacture having a coating of metal thereon produced by an electrolytic deposition process involving the use of the usual electrolytic pair, and an independent electrode of non-resolvable character inserted in an electric circuit of different characteristics conveyed to the electrodes through the electrolyte.

14. An article of manufacture having a coating of metal thereon produced by an electrolytic deposition process involving the use of the usual electrolytic pair and an independent electrode inserted in an electric circuit of different characteristics conveyed to the electrodes through the electrolyte.

HARRY D. GUE.